

May 30, 1967

MIKIO ASHIKAWA ET AL

3,322,570

PHOTORESPONSIVE ELECTRODES AND METHOD OF MAKING SAME

Filed May 21, 1963



FIG. 1



FIG. 2

INVENTORS  
MIKIO ASHIKAWA  
HIDEKI UMEZAWA  
KAZUO OZAWA  
BY  
Paul M. Craig, Jr.  
ATTORNEY

1

**3,322,570**  
**PHOTOSENSITIVE ELECTRODES AND METHOD**  
**OF MAKING SAME**

Mikio Ashikawa, Tokyo, Hideki Umezawa, Hachioji-shi, Tokyo, and Kazuo Ozawa, Tokyo, Japan, assignors to 5 Hitachi, Ltd., Tokyo, Japan, a corporation of Japan

Filed May 21, 1963, Ser. No. 281,959

Claims priority, application Japan, May 25, 1962,  
37/20,917

7 Claims. (Cl. 117—211)

This invention relates generally to photoconductive layers and more particularly to photosensitive electrodes for Vidicon and other pickup tubes and methods of making such electrodes.

In the past, photosensitive electrodes of the kind described have generally included a composite layer including a first and porous layer of photoconductive material vapor-deposited on the electrically conductive substrate in the atmosphere of low pressure gas and a second and solid, glassy layer of photoconductive material vapor-deposited on the first layer in vacuum or one comprised of three successively superposed layers including a first and a second solid layer with a porous layer therebetween. Porous layers are characterized by their extremely high electrical resistivity and fast photoresponse but are usually low in photosensitivity. In contrast, solid layers generally have a photosensitivity higher than that of porous layers but are slow in photoresponse and lower in electrical resistivity. Thus the use of a composite layer comprised of two or three elementary layers as described above has been for the purpose of obtaining a photosensitive electrode having satisfactory characteristics as a whole by allowing the porous and solid layers to have their demerits offset by each other.

However, since the characteristics of such composite layer are largely influenced by the magnitude and proportion of the thicknesses of the respective elementary layers, the gas pressure under which the porous layer is vapor-deposited and other factors, it has been difficult to obtain a composite layer having desired stable and constant characteristics.

The present invention is intended to provide a photosensitive electrode which includes a single-layer apparently easier to form than any multiple composite layer and has characteristics at least compatible to those of any conventional photosensitive electrode, which has a multiple-layer and to provide a method of making such photosensitive electrode having a single-layer.

According to the method of the present invention, the vapor deposition of a photoconductive material is performed in a gaseous atmosphere while varying the pressure thereof in a continuous fashion from a high to a low vacuum or vice versa to obtain a photosensitive electrode comprised of a vapor-deposited photoconductive layer varying continuously in porosity through the thickness of the layer.

It will be appreciated that the electrode made according to the present invention includes a photoconductive layer which is apparently a single-layer but has characteristic properties combining the merits of a porous and a solid film. In addition, such characteristic properties can be controlled with ease by controlling the rate at which the gas pressure is varied.

The present invention will now be described in further detail by a practical example of the typical procedure in connection with the accompanying drawings, in which:

FIGURE 1 illustrates a portion of a pick-up tube employing a photosensitive electrode according to the present invention, and

FIGURE 2 illustrates a characteristic performance 70 of the photosensitive electrode according to the present invention.

2

In FIGURE 1, there is shown a tubular glass envelope 1 and at one end of this envelope 1 a photosensitive electrode 2 which according to this invention is hermetically sealed to envelope 1 through a metal ring 6.

The photosensitive electrode 2 also serves as a window for the envelope 1 and comprises a transparent substrate 3 such as a glass plate having a transparent, electrically conductive layer 4, for example, a tin oxide layer, coated on the inner surface of the substrate 3 and a single layer 5 of photoconductive material such as antimony trisulfide, vapor-deposited on said conductive layer 4.

Adjacent to and facing the inner surface of the photosensitive electrode 2, but at a slight distance therefrom, is provided a metal mesh electrode 7 carried by a metal cylinder 8.

A practical example for making the photosensitive electrode according to the present invention is as follows. In this example, it is assumed that antimony trisulfide is employed as a photoconductive material and argon as an ambient gas. A substrate made of glass plate carrying a transparent electrically conductive layer on one surface of said glass plate and antimony trisulfide being contained in a crucible is first placed in a vacuum evaporation unit. Then the unit is evacuated and the crucible is heated to 20 evaporate antimony trisulfide. The time requirement for the vapor deposition of antimony trisulfide is measured in advance, which is usually a few minutes. The opening of the gas valve in the argon gas inlet section is positioned and the throttle in the gas inlet conduit is set in accordance with the time requirement. Thus, in case the deposition time required is, for example, five minutes, the argon gas inlet section is set up so that the pressure in the evaporation unit is varied from  $10^{-5}$  mm. Hg to  $10^{-1}$  mm. Hg in five minutes. In this case, if the pressure in the evaporation unit is varied in proportion to the time elapsing after the vapor-depositing has been started, the layer vapor-deposited on the substrate will have a porosity linearly varying through the thickness of the layer, ranging from an extremely compact solid structure obtained under the pressure of  $10^{-5}$  mm. Hg, to a porous structure obtained under the pressure of  $10^{-1}$  mm. Hg.

One example of the characteristic performance of the photosensitive electrode is illustrated in FIGURE 2. The illustration represents the so-called light transfer characteristics of Vidicon tubes, which clearly expresses the sensitivity of the tubes. In the drawing, the abscissa represents the intensity of illumination on the surface of the photosensitive electrode while the ordinate represents the magnitude of the signal output current of the Vidicon, both in a logarithmic scale. The signal output current has been determined for a predetermined dark current of 0.02  $\mu$ A. for each Vidicon.

Also in FIGURE 2, lines 1, 2 and 3 illustrate the characteristics of respective Vidicons employing a photosensitive electrode of the present invention, one including a three-layer, layer, and one including a two-layer, layer, respectively.

At present, it is generally considered that the best way of comparing the sensitivity between Vidicons is to determine the intensity of illumination on the surface of the photosensitive electrode as required to allow the Vidicon to provide a signal output of a specific current value. As will be observed in the chart, the values of the intensity of illumination determined from lines 1, 2 and 3 for a signal output current of 0.1  $\mu$ A. are 0.35 lux, 2.8 lux and 18 lux, respectively. In other words, the light requirement of the photosensitive electrode made according to the present invention is about one-eighth of that of the three-layer, layer electrode and about  $\frac{1}{16}$  of that of the two-layer, layer electrode, that is, the inventive photosensitive electrode has a highly improved sensitivity, which is about

eight times and fifty-one times as high as that of the three- and two-layer film electrodes, respectively.

Moreover, it will be apparent from the foregoing that the variation in porosity of the photoconductive layer through its thickness can be otherwise controlled by varying the gas pressure in the evaporation unit at an appropriate rate instead of varying the pressure in proportion to time.

Thus, it will be seen that in the practice of this invention a photoconductive layer having a porosity varying through its thickness in any desired manner can be obtained by controlling the variation in pressure of the gasous atmosphere within the evaporation unit. Accordingly, in the practice of the invention, the relationship between the photosensitive electrode performance and the manufacturing method can be determined easily compared with the case of conventional photosensitive electrode having two- or three- composite layers of photoconductive material. Thus it is possible to make photosensitive electrodes which are improved in performance over conventional ones.

What we claim is:

1. A photosensitive electrode comprising a transparent substrate having a transparent, electrically conductive layer on one surface thereof and a single layer of photoconductive material disposed on said electrically conductive layer, said photoconductive material having a porosity which varies continuously from the solid state to the porous state or from the porous state to the solid state through the thickness of the photoconductive layer.

2. A photosensitive electrode according to claim 1, wherein the porosity varies continuously and linearly or randomly from the solid state to the porous state or from the porous state to the solid state through the thickness of the photoconductive layer.

3. A photosensitive electrode according to claim 1,

wherein said photoconductive layer is antimony trisulfide.

4. A method of making a photoconductive electrode which comprises placing a transparent substrate having a transparent, electrically conductive layer in an evaporation unit with a photoconductive material, and heating the photoconductive material to evaporate it while varying the pressure in said evaporation unit gradually from a first predetermined value to a second predetermined value which is higher or lower than said first predetermined value, to cause deposition of a single layer of photoconductive material on the surface of said electrically conductive layer, said photoconductive material having a porosity varying continuously through the thickness of the photoconductive layer.

5. The method of claim 4, wherein the porosity varies continuously and linearly or randomly from a solid state to a porous state, or from a porous state to a solid state through the thickness of the photoconductive layer.

6. The method of claim 4, wherein said photoconductive material is antimony trisulfide.

7. The method of claim 4, wherein the pressure is varied from about  $10^{-5}$  mm. Hg. to  $10^{-1}$  mm. Hg.

#### References Cited

##### UNITED STATES PATENTS

|           |        |            |       |           |
|-----------|--------|------------|-------|-----------|
| 2,967,962 | 1/1961 | Turk       | ----- | 117—106 X |
| 3,015,746 | 1/1962 | Lubszynski | ----- | 313—65    |

##### FOREIGN PATENTS

|         |        |         |
|---------|--------|---------|
| 138,950 | 8/1960 | Russia. |
|---------|--------|---------|

ALFRED L. LEAVITT, Primary Examiner.

35 WILLIAM L. JARVIS, Examiner.